

## UNITED STATES PATENT OFFICE

WALLACE B. VAN ARSDEL, OF BERLIN, NEW HAMPSHIRE, ASSIGNOR TO BROWN COMPANY, OF BERLIN, NEW HAMPSHIRE, A CORPORATION OF MAINE

ARTIFICIAL LEATHER FABRICATION

No Drawing. Application filed September 30, 1929. Serial No. 396,412.

This invention relates to the fabrication of artificial leather, more particularly of the type comprising a foundation of interfelted cellulose fibers impregnated throughout with rubber. Such a product is useful in making various articles, such as shoes, upholstered furniture, automobile tops, traveling bags, and the like. It has been found that a porous web of interfelted cellulose fiber made on machinery of the papermaking type serves well as the foundation material, particularly when it is desired that the resulting product have characteristics closely simulating those of natural leather. When a web of the character described is impregnated with a rubber-carrying vehicle such as the so-called rubber solutions in organic solvents, or aqueous dispersions of rubber, and the liquid vehicle then removed, the resulting product has high flexibility, tensile strength, and tear resistance, and is resilient and of sufficient porosity to be used in the manufacture of innersoles which permit breathing of the foot and which absorb perspiration therefrom. In some methods of shoemaking, it is desired to dispense with a so-called sock lining on the innersole, but where this is done, the inner surface of the innersole should be finished to provide good appearance and suitable feel to the foot. When artificial leather such as described is finished and embossed to produce the desired appearance and feel, under the heavy pressure employed in embossing it becomes so compacted and loses so much resiliency and porosity as to be unacceptable for the purpose desired.

In accordance with the present invention, I produce an artificial leather from a plurality of rubber-impregnated plies of interfelted cellulose fiber, a surface ply being suitably finished and embossed before being bonded with the other ply or plies. By finishing and embossing only a surface ply which may be a comparatively thin sheet, it is possible to produce a product having not only the desired appearance and feel but also having the resiliency and porosity desired in such articles as innersoles.

In producing the artificial leather of the present invention, I prefer to use a highly

porous web of loosely felted cellulose fiber as the foundation material, for, when such a web is impregnated with a suitable rubber-carrying liquid vehicle, upon the removal of the liquid vehicle, the rubber serves to bind together strongly the fibers of the foundation, and at the same time sufficient porosity is restored thereto so that it is resilient and capable of readily absorbing moisture. Preferably, the rubber-impregnated web to serve as the surface ply of the finished product is of lower rubber content than the other ply or plies, so that after this ply is finished with suitable materials such as lacquers, and then embossed, it will have greater porosity than were a ply of higher rubber content employed. In making an artificial leather for use in the manufacture of innersoles, the surface ply may have a rubber content of, say, about 70% to 90%, based on fiber, whereas the other ply or plies may have a rubber content of, say, about 100% to 200%, also based on fiber. The use of plies of different rubber content in the production of an artificial leather to be used in the manufacture of innersoles is not, however, my sole invention, this feature being disclosed and claimed in application Serial No. 395,744, filed September 27, 1929, by George A. Richter and myself.

A procedure which may be followed in producing the product of the present invention, may be substantially as follows. A fluffy web composed of loosely interfelted cellulose fibers and possessing high porosity is preferably used as the foundation material for all the plies. A web of unusually high porosity may be produced by using a substantially unbeaten wood fiber of high alpha cellulose content, say, 94% or greater, as a raw material, and forming such fiber into a web on a papermaking machine designed to effect dewatering and drying of the web without the application of the heavy pressures used in ordinary papermaking practice. While other fibers in substantially unbeaten condition, such as sulphite, kraft, or soda pulp, may be employed, a substantially unbeaten wood fiber of high alpha cellulose content is preferred, because it is more highly absorp-

tive than the usual unbeaten commercial persion, so that the dried, rubber-impregnated web may be vulcanized under the wood fibers, and hence enhances the absorptivity or porosity resulting from the loosely action of heat, if desired. felted, uncompact condition of the fibers. The dry, porous web may be passed through 5 a bath of rubber-carrying vehicle such as an ammonia-preserved latex of a solids content of, say, about 16%, at which content immersion for about five to thirty seconds effects a thorough impregnation of the web. If to be used as the surface ply of the sole, the impregnated web may be squeezed until its rubber solids content is about 70% to 90%, based on the weight of dry fiber, and if to be used as the other plies, until its rubber 10 solids content is about 100% to 120%. In order to prevent migration of the rubber globules to the surface of the web during drying, the ammonia-preserved latex may be treated with the oxide of an amphoteric 15 metal, preferably zinc oxide, as described in application Serial No. 369,267, filed June 7, 1929, by Roger B. Hill, or with alkaline earth metal hydroxides, preferably slaked lime, as described in application Serial No. 373,055, 20 filed June 22, 1929, by Roger B. Hill. When slaked lime is the compound added to the latex to overcome migration tendencies during drying, protective colloids such as soluble 25 soaps or caseinates which are capable of being precipitated by lime as insoluble calcium soaps or caseinates, are preferably added to the latex prior to the addition of the slaked lime, in order to overcome coagulating 30 tendencies. Such treatment of the latex prior to its use for the impregnation of the web makes possible the production of a dried, rubber-impregnated web of uniformity in respect of rubber distribution therethrough, as 35 troublesome non-rubber constituents of the latex, namely, the proteins and the resins, are converted to an insoluble, inert condition. Apparently, setting or coagulation of the rubber by drying is so retarded by the proteins and resins which exist respectively in 40 an ammonia-preserved latex as water-soluble proteinates and alkali resinates, that there is a tendency for rubber particles to migrate to the surface of the impregnated product, 45 where evaporation of water is taking place. The tendency for migration of rubber particles is especially pronounced in the case of highly porous webs of cellulose fiber of the type described, evidently because of the high 50 capillary action taking place during drying to cause such migration.

If desired, a vulcanized latex may be used, so that when the latex-impregnated web is subsequently dried, the rubber will be coagulated in the web in vulcanized condition. Or artificial aqueous dispersions may be used 55 in lieu of natural latex. Suitable rubber-compounding materials, vulcanizing agents, and accelerators of vulcanization may be added to the artificial or natural rubber dis-

The web used as a foundation material for all the plies is preferably comparatively thin. In actual practice, a web of about 100 pounds basis weight (i. e., the weight of 2880 sq. ft. of web) may be employed to good advantage. The impregnated web is of insufficient thickness for the manufacture of products such as innersoles, so that it is necessary to bond together two or more webs. In accordance with the present invention, the impregnated web to be used as the surface ply is suitably finished and embossed prior to bonding with one or more other webs into a finished product of the desired thickness. To this end, a single web impregnated to a rubber content of preferably about 70% to 90% may be finished according to the color, gloss, grain, and wearing qualities desired. The most durable of the finishes with which I am familiar are the nitro-cellulose lacquers, as they impart gloss and smoothness to the sole and are permanent against the action of perspiration. The lacquer may be applied to the surface of the web as by spraying, whereupon the coated product may be dried. The lacquered surface may then be embossed under heavy pressures, to produce grain effects simulating those of natural leather, the finished and embossed ply being of much greater compactness than the original rubber-impregnated web. The finishing and embossing treatment may include additional steps to ensure a finish of sufficient thickness and covering power. For instance, an initial or base coat of clear nitro-cellulose lacquer may be applied to the surface of the sheet, whereupon one or more coats of nitrocellulose lacquer containing suitable pigments or fillers may be applied. The base coat prevents sinking of the pigments or fillers into the rubber-impregnated foundation, where they are undesirable. The lacquered and pigmented surface may then be embossed and a final coat of clear nitrocellulose lacquer may be applied thereto. The lacquered surface may then be smooth-plated to destroy the oily or greasy appearance and to bring out the gloss.

If desired, so-called water finishes may be used in lieu of nitrocellulose lacquers, these finishes consisting generally of alkaline solutions of shellac, and yielding coatings which, although of less durability than nitrocellulose lacquer coatings, are of greater porosity. The finished sheet may then be embossed, as previously described.

The finished embossed sheet may then be bonded with one or more other sheets having a rubber content of about 100% to 120%, a rubber adhesive such as latex preferably being used as the bonding material. It has been found advantageous to moisten the wet

surfaces of the dried, rubber-impregnated sheets, and then to apply comparatively thick, concentrated latex as the bonding material, whereupon the sheets may be superposed, united under comparatively slight pressure, and dried. Apparently the initial moistening or setting of the plies promotes penetration of the thick latex into the surface portion of the plies, and results in a better interlocking or bonding together of the plies in face-to-face relationship after the latex is dried. The resulting product may be cut into innersoles or other shoe parts, or be used for any other articles where characteristics such as possessed thereby are desired.

I claim:

1. An artificial leather product comprising a plurality of rubber-impregnated plies of cellulose fibers, the surface ply only being finished and embossed and having greater compactness than the rest of the product.
2. A method which comprises finishing and embossing a porous, rubber-impregnated web of interfelted cellulose fibers, bonding it as a surface ply with one or more other porous, rubber-impregnated webs of interfelted cellulose fibers, and cutting into innersoles.
3. An artificial leather product comprising a plurality of rubber-impregnated plies of cellulose fibers, including a relatively thin surface ply, said surface ply only being finished and embossed and having greater compactness than the rest of the product.

In testimony whereof I have affixed my signature.

WALLACE B. VAN ARSDEL.

40

45

50

55

60

65